

## UNITED STATES PATENT OFFICE.

ARTHUR GEORGE HARRINGTON, OF LONDON, ENGLAND, ASSIGNOR OF ONE-HALF TO  
HAROLD LIONEL BRANDON, OF LONDON, ENGLAND.

## WATERPROOFING OF FABRIC ARTICLES.

No Drawing.

Application filed December 1, 1924. Serial No. 753,338.

*To all whom it may concern:*

Be it known that I, ARTHUR GEORGE HARRINGTON, a subject of the King of England, residing at London, England, have 5 invented certain new and useful Improvements in Waterproofing of Fabric Articles, of which the following is a specification.

This invention consists of improvements in or relating to the waterproofing of fabric 10 articles.

It is in many instances desirable to render waterproof an article which is made of woven fabric after its manufacture has been completed in other respects.

15 With certain articles of fabric, stitching during manufacture renders the article pervious to water in places, even although the original fabric were waterproofed. For example in the manufacture of motor-car 20 hoods, the stitching of the sections may give rise to leaky places.

According to the present invention articles of woven fabric made up by stitching are waterproofed in finished form by applying a solution of paraffin wax in a volatile solvent. It is found that this renders 25 stitching and fabric simultaneously waterproof without adversely affecting the appearance of the goods.

30 The invention will be described by way of example in its application to two articles.

A motor-car hood is made up by stitching in any ordinary way, and either before 35 or after use it is found not to be waterproof. Hard paraffin is dissolved in a volatile solvent, such as benzene or petrol, with or without material to render the same noninflammable (such as trichlorethylene). 40 It is preferable that the solution should be made concentrated, or nearly concentrated at a low normal atmospheric temperature, such as 40° F. The solution is painted on to the fabric, and the solvent evaporates, 45 leaving a thin coating of hard paraffin on the fibres and threads constituting the fabric.

In the manufacture of ornamental bathing caps, it is desirable that the maker 50 should be free to use any desired materials or combination of materials, and make them up into finished form from fabrics (not

necessarily waterproof fabrics) chosen on account of their quality and colours. Articles thus made up are immersed in the solution of hard paraffin above referred to, and then removed from the solution, whereupon the volatile solvent evaporates and leaves the article in the waterproof condition the lines of stitching being rendered completely 60 leakproof.

In articles of this kind a further advantage of the invention arises from the fact that where an article is made of coloured fabric or of fabric containing a variety of 65 colours or of a variety of fabrics of different colours, it may be difficult, if not impossible, to apply the desired colours to fabrics which have already been rendered waterproof, and some known methods of 70 waterproofing would impair the colours.

An article not ordinarily waterproofed, e. g. a fancy sunshade or cloak may be treated, so as to be waterproof against a sudden shower of rain. Waterproof articles, such as awnings, or hatch coverings for 75 ships, which have been patched with new material, can be treated at the patching, while old material which has lost its waterproof qualities through time or exposure to 80 heat or damp, the fibres remaining good, can be re-proofed in situ by the treatment.

The preferred way of making up the solution is first to melt up the hard paraffin wax with a small proportion, say 0.5% by 85 weight of essential oil of citronella and a small proportion of a fat-soluble dye, for example a brown dye (just sufficient to give a brown coloration). The mixture is allowed to solidify and is then shredded into 90 small flakes in which condition it can readily be transported; these flakes are dissolved in petrol which may contain a small proportion say 1% of trichlorethylene, in the proportion of 6 oz. of flakes to 1 gallon 95 of solvent. This solution is applied to the articles of fabric or the like, and any excess solution may be drained off. The solvent evaporates and leaves the article in a waterproofed state.

100 It will be understood that according to this invention finished articles of woven material are treated after they have been stitched together so that stitching and

woven material are both simultaneously rendered waterproof.

I claim:—

5 A composition for waterproofing fabrics including hard paraffin wax dissolved in petrol to which a small proportion of tri-chlorethylene has been added.

In testimony whereof I have signed my name to this specification in the presence of two subscribing witnesses.

ARTHUR GEORGE HARRINGTON.

Witnesses:

HUGH S. MACEAU,  
S. G. PEVERO.